

# UNITED STATES PATENT OFFICE.

JOHN M. BURBY, OF WEBSTER, MASSACHUSETTS.

## PROCESS OF REPULPING OLD OR WASTE PAPER.

1,327,590.

Specification of Letters Patent.

Patented Jan. 6, 1920.

No Drawing.

Application filed April 14, 1916. Serial No. 91,213.

*To all whom it may concern:*

Be it known that I, JOHN M. BURBY, a citizen of the United States, residing at Webster, in the county of Worcester and 5 State of Massachusetts, have invented a new and useful Process of Repulping Old or Waste Paper, of which the following is a specification.

This invention relates to a process of 10 repulping old or waste paper and particularly to a process for making a high grade chemical pulp from old news print or other similar grades of paper.

In the manufacture of paper pulp from 15 wood, several different processes are used. The better grades of pulp are known to the trade as chemical pulp and are made by subjecting small chips or pieces of wood to the action of certain chemicals which dissolve 20 the pitch and other binding materials which hold the wood fibers together, thereby freeing the fibers so that they may be readily matted or felted together. From this chemical pulp the better grades of paper are manufactured and these papers are practically 25 free from raw or undigested wood.

The pulp from which news print and other cheap papers are made is termed mechanical wood pulp and is made by grinding 30 the raw wood to small particles which are thereafter washed and graded and then collected to form sheets of convenient size. This pulp is much inferior to the chemical pulp in strength and can only be used for 35 very cheap grades of paper, as the raw wood particles change color upon exposure to light. Even when so used it is commonly necessary to add a certain percentage of chemical pulp in order to produce a workable paper.

News print and other papers formed from mechanical wood pulp contain from forty to ninety per cent. of raw or undigested ground wood and it is not possible to repulp such 45 papers by any process heretofore known, in such a manner as to produce high grade paper therefrom.

It is the object of my present invention to provide a process by which a high grade 50 chemical pulp may be made from news print or other cheap papers containing a large amount of raw wood.

With this object in view my invention relates to a certain sequence of operations by 55 which the old paper and the raw or ground

wood contained therein may be transformed into chemical pulp.

In the carrying out of my improved process, the old paper is first reduced to pieces of convenient size by means of well-known machines customarily used for this purpose.

If a particularly light-colored and high grade pulp is desired, it may be advisable to 60 subject the paper to the action of an alkaline solution, in order to remove the ink and coloring matter therefrom, this action taking place at a comparatively low temperature and never above the boiling point of water 65 212° F.

This preliminary treatment, while often 70 desirable, is not an indispensable step in my process, as a very satisfactory pulp for many purposes can be made without the preliminary alkaline treatment.

In the further carrying out of my process 75 the waste paper, either untreated or treated with alkali as above described, is placed in a solution of suitable chemicals and is boiled therein for a period of time sufficient to permit these chemicals to convert the raw or ground wood fibers into chemical pulp. I have found that a considerable range of 80 chemicals may be used for attaining this result, and the selection of chemicals depends largely upon the grade or kind of chemical 85 pulp desired.

I secure a better grade of pulp by boiling 90 the waste paper in a solution containing bisulfite of calcium, magnesium or sodium, the pulp thus obtained corresponding to the so-called sulfite pulp of commerce and possessing strong fibers firmly matted or felted together. This pulp is very light in 95 color and may be used with or without supplementary bleaching in the production of high grade book papers.

By boiling the old paper in a solution containing sodium sulfate, with or without 100 the addition of caustic soda and sodium carbonate, I secure a pulp of darker color corresponding to the so-called sulfate pulp or kraft of commerce.

While I have attained good results by the use of the chemicals named, I do not wish 105 to be understood as limiting my process to the use of any particular chemicals except as set forth in the claims, as I have also attained good results from the use of sodium sulfid and also by the use of other chemical 110

mixtures containing sodium, sulfur and lime in different forms and proportions. The essential feature is that the chemicals, when used at a temperature above 212° F., should 5 be effective to digest the raw wood of the news print and other cheap papers, and to transform the same into a strong chemical pulp.

The period of time necessary for this 10 treatment varies with the chemicals used, and under ordinary circumstances will be from four to eight hours. The action of the chemicals is more rapid and the time is reduced if the boiling process is carried out 15 in a suitable closed tank or digester under pressures which may run as high as seventy or eighty pounds or more.

After the boiling process is completed, the 20 pulp is removed and may then be sent through a beating engine by which the fibers are torn apart and the pulp is thoroughly washed. The pulp is then removed for bleaching if desired and is finally collected 25 and passed under rollers by which it is pressed into sheets convenient for shipment and handling.

The chemical pulp thus obtained is suitable for any of the purposes to which similar 30 pulp made from wood chips may be applied, the character of the pulp depending somewhat upon the chemicals used as above described.

The ground wood contained in old paper 35 is more accessible to the action of the digesting solution than is wood in the form of blocks or chips. The solution may therefore be of much less strength and the time required for boiling is also correspondingly less. When carried out in this way the cost 40 of the solutions is merely nominal.

Having thus described my invention in detail, it will be evident that other changes and modifications can be made therein by those skilled in the art without departing from the spirit and scope thereof as set 45 forth in the claims and I do not wish to be otherwise limited to the details herein disclosed, but what I do claim is:—

1. The process of converting old paper made from mechanical wood pulp into 50 chemical wood pulp by boiling said paper in a solution containing chemicals effective to act upon the mechanical wood pulp of the old paper and to reduce said wood pulp to the nature of a chemical wood pulp. 55

2. The process of converting old paper containing ground wood into chemical wood pulp by boiling said old paper in a digester under pressure above atmospheric, said digester containing chemicals effective to 60 act upon the ground wood of the old paper and to reduce said paper to the nature of a chemical wood pulp.

3. The process of converting old paper containing ground wood into chemical wood 65 pulp by boiling said old paper in a solution of chemicals containing sulfur, in a form effective to reduce the ground wood of the old paper to the nature of a chemical wood pulp. 70

4. The process of converting old paper containing ground wood into chemical wood pulp, which consists in boiling said old paper in a bisulfite solution of sufficient strength to change the old paper into chemical wood 75 pulp.

In testimony whereof I have hereunto set my hand.

JOHN M. BURBY.